

## UNITED STATES PATENT OFFICE

2,416,909

## FROTH FLOTATION OF PHOSPHATE ORE

Bruce Donaldson Crawford, Greenwich, and  
 David Walker Jayne, Jr., Old Greenwich, Conn.,  
 assignors to American Cyanamid Company,  
 New York, N. Y., a corporation of Maine

No Drawing. Application May 13, 1942,  
 Serial No. 442,818

4 Claims. (Cl. 209—166)

1

This invention relates to an improved method for the froth flotation of phosphate ores using the so-called anionic flotation agents.

The problem of beneficiating phosphate rock by froth flotation methods is considerably complicated by the fact that the phosphate is a relatively low priced material and that the flotation operation results in floating a relatively large weight of material in the form of a concentrate. There is no problem at all in floating most phosphate rock qualitatively. Any of the common flotation agents for non-metallic materials such as fatty acids and fatty acid soaps will float phosphate, but in order to achieve a commercial result it is necessary to obtain a high grade of concentrate as a relatively large premium is paid for grade. At the same time, this result must be obtained with a reasonable reagent cost and with a fair degree of recovery.

It was found that when soaps were used to float phosphate rock, results were not satisfactory. The next development was to use fatty acids, caustic alkali and hydrocarbon or other non-saponifiable diluents. This procedure resulted in a commercial process which is used almost exclusively in the Florida Pebble Phosphate field. Further improvements resulted when fatty acids were substituted by talloel which is a mixture of unsaturated aliphatic acids and rosin acids, and this combination of reagents represents the best commercial efficiency achieved with the caustic alkali hydrocarbon oils and acid process.

The present invention is a departure from the procedure which was finally worked out after years of investigation and goes back in part to the use of a type of reagent which was considered unsatisfactory for phosphate flotation, namely the use of soaps instead of the free acids admixed with caustic alkali so as to form compounds in situ. It was found that if instead of using a non-saponifiable diluent such as fuel oil, a saponifiable oil which is the ester of a polyhydric alcohol and one or more fatty acids or liquid free fatty acid gives improved recoveries, particularly in the case of feed which has been freed from both primary and secondary slimes.

In using the process of the present invention it should be noted that there are some differences in the optimum amounts of the promoter which should be used. In general, the soaps will require a larger amount than free fatty acids when used with fuel oil. Comparisons on the basis of

2

the same amount are therefore misleading because if as little soap is used as is equivalent to the fatty acid in the fuel oil process, the recoveries will be unsatisfactory, whereas if as much fatty acid is used with fuel oil as soap with saponifiable oil, the grade is uncommercial. Therefore in comparative tests which will be shown in some of the specific examples to follow, each type of reagent has been used in its optimum amount in order to obtain the best possible results with each reagent.

Not only is there a difference between the amount of soap and the amount of free fatty acid to be used to obtain best results, but results will vary somewhat with different soaps and of course in every case the best proportions will be used.

It might be expected that a saponifiable oil in the form of an ester will behave differently than a saponifiable oil in the form of a free fatty acid.

It would normally be expected that in the latter case the free fatty acid would act as a promoter, which role it plays in processes using fuel oil associated with fatty acid. This, however, appears not to be the case because talloel which is

a mixture of fatty acids and rosin acids may be used interchangeably with saponifiable esters such as coconut oil and the like. The reason for this surprising behavior has not been determined

exactly but it seems probable that promoter action may be tied up in some way with the amount of alkali present and that only the soap acts as a promoter, the unsaponified fatty acid behaving in a different manner, whereas when larger amounts of free fatty acids are used with fuel oil, larger amounts of soap are formed because the alkali is also present in such a process in large excess over the molecular equivalent to the fatty acid used.

A further practical advantage of the process of the present invention is that it is relatively insensitive to changes in amount of collector within fairly wide limits. While there is, of course, an optimum amount of collector for each particular ore and for each particular collector, nevertheless the amounts may be varied throughout a considerable range, which range is much broader than in the case of the known caustic soda, fatty acid, fuel oil process. This insensitivity to

changes in amounts of reagents is of considerable value in practical phosphate flotation as it removes a critical factor. Phosphate feed and

other conditions in the flotation plant will vary to some extent from day to day and hour to hour and it is advantageous to obtain uniformly good results even with considerable variation in conditions, thus making a continuous expert supervision less necessary.

The invention will be described in greater detail in conjunction with the following specific examples.

#### EXAMPLE 1

A typical phosphate feed from the Florida Pebble Phosphate district having between 35 and 36%

fuel oil and 0.342 pound per ton of talloel. The reagents were added in the order given while the mixer was continuously operating. The pulp was diluted to flotation consistency and subjected to 5 froth flotation in a Fagergren flotation machine as described in Example 1.

A further portion of feed was conditioned in the same manner but using 0.25 pound per ton caustic soda, 0.63 pound per ton of talloel and 10 4.00 pounds per ton of #2 fuel oil. Conditioning, dilution and flotation were the same as above. The metallurgical results appear in the following table:

Table II

|                     | Per cent wt. | Assays |        | Percent distribution |        | Lbs./ton feed |          |         |
|---------------------|--------------|--------|--------|----------------------|--------|---------------|----------|---------|
|                     |              | Insol. | B.P.L. | Insol.               | B.P.L. | NaOH          | Fuel oil | Talloel |
| Cleaned concentrate | 40.68        | 6.75   | 74.67  | 4.97                 | 86.80  | 0.318         | 1.794    | 0.342   |
| Middling            | 8.96         | 73.64  | 21.32  | 11.92                | 3.40   | .318          | 1.794    | .342    |
| Rougher tailing     | 50.36        | 91.40  | 6.82   | 83.11                | 9.80   | .318          | 1.794    | .342    |
| Feed                | 100.00       | 55.38  | 35.00  | 100.00               | 100.00 |               |          |         |
| Cleaned concentrate | 44.28        | 9.73   | 71.82  | 7.90                 | 88.75  | .250          | 4.000    | .630    |
| Middling            | 10.22        | 82.98  | 13.22  | 15.57                | 3.77   | .250          | 4.000    | .630    |
| Rougher tailing     | 45.50        | 91.62  | 5.89   | 76.53                | 7.48   | .250          | 4.000    | .630    |
| Feed                | 100.00       | 54.48  | 35.83  | 100.00               | 100.00 |               |          |         |

B.P.L. was conditioned at 70% solids with 0.88 pound per ton of saponified talloel (sodium salts) and one pound per ton of coconut oil. The pulp was then diluted to 22% solids and subjected to froth flotation in a Fagergren flotation machine, the rougher concentrate being collected after short further conditioning.

The same feed was conditioned with 0.88 pound per ton of saponifiable talloel and two pounds per ton of coconut oil and subjected to the same flotation procedure. The metallurgical results are shown in the following table:

Table I

|                     | Per cent wt. | Assays |        | Percent distribution |        | Lbs./ton feed<br>coconut oil |
|---------------------|--------------|--------|--------|----------------------|--------|------------------------------|
|                     |              | Insol. | B.P.L. | Insol.               | B.P.L. |                              |
| Cleaner concentrate | 40.25        | 4.17   | 73.94  | 3.04                 | 85.66  | 1.00                         |
| Middling            | 4.79         | 49.72  | 38.59  | 4.37                 | 5.33   | 1.00                         |
| Rougher tailing     | 54.98        | 91.82  | 5.70   | 92.59                | 9.01   | 1.00                         |
| Feed                | 100.00       | 54.50  | 34.74  | 100.00               | 100.00 |                              |
| Cleaner concentrate | 44.12        | 6.26   | 73.05  | 5.04                 | 92.04  | 2.00                         |
| Middling            | 2.83         | 75.52  | 18.86  | 3.91                 | 1.51   | 2.00                         |
| Tailing             | 53.05        | 93.94  | 4.26   | 91.05                | 6.45   | 2.00                         |
| Feed                | 100.00       | 54.74  | 35.02  | 100.00               | 100.00 |                              |

It will be apparent that the grade obtained is relatively insensitive to large increases in the amount of coconut oil used and high recovery is obtained thereby with only a small sacrifice in grade.

It will be apparent that the addition of further amounts of fuel oil while it did somewhat raise the recovery, did have disastrous effects on the grade, the amount of insoluble material becoming so high as to be commercially useless.

#### EXAMPLE 3

35 A high grade Florida pebble phosphate feed having from 43 to 45% of B.P.L. was conditioned with a mixture of the sodium soap of talloel and unsaponified talloel under the conditions described in Example 1, and was subjected

Table III

| Feed   |      | Concentrates |        |      | Middlings |      | Tailings |      | Ratio | Recov. | Reagents, lbs./ton feed |         |
|--------|------|--------------|--------|------|-----------|------|----------|------|-------|--------|-------------------------|---------|
| B.P.L. | Gms. | B.P.L.       | Insol. | Gms. | B.P.L.    | Gms. | B.P.L.   | Gms. |       |        | Talloel soap            | Talloel |
| 43.81  | 511  | 79.03        | 3.71   | 239  | 68.02     | 31   | 5.77     | 241  | 2.14  | 84.3   | 0.44                    | 1.68    |
| 43.84  | 510  | 77.49        | 5.42   | 264  | 37.29     | 29   | 3.78     | 217  | 1.93  | 91.6   | .88                     | 1.12    |
| 43.08  | 518  | 77.45        | 4.41   | 259  | 62.23     | 19   | 4.46     | 240  | 2.00  | 89.9   | .32                     | 1.51    |
| 44.32  | 515  | 78.20        | 3.66   | 245  | 68.78     | 27   | 7.45     | 243  | 2.10  | 84.0   | .22                     | 1.51    |
| 44.92  | 514  | 80.09        | 3.79   | 234  | 72.63     | 35   | 7.36     | 245  | 2.20  | 81.0   | .11                     | 1.51    |

#### EXAMPLE 2

The phosphate feed of Example 1 was conditioned in the same manner but using 0.318 pound per ton caustic soda, 1.794 pounds per ton #2

55 to flotation as there described. The feed was sized -20 +65 mesh. Various proportions of talloel soap and talloel were used and the results for the different proportions appear in the following table of metallurgical results:

#### EXAMPLE 4

Feed of the type described in Example 3 was conditioned with various amounts of sodium soap of talloel and coconut oil and floated as described

in the above example. The following table shows the metallurgical results: talloel soap per ton of feed and 1.13 pounds of talloel per ton of feed and floated as described

Table IV

| Feed   |      | Concentrates |        |      | Middlings |      | Tailings |      | Ratio | Recov. | Reagents, lbs./ton feed |             |
|--------|------|--------------|--------|------|-----------|------|----------|------|-------|--------|-------------------------|-------------|
| B.P.L. | Gms. | B.P.L.       | Insol. | Gms. | B.P.L.    | Gms. | B.P.L.   | Gms. |       |        | Talloel soap            | Coconut oil |
| 43.78  | 525  | 80.85        | 2.45   | 172  | 72.87     | 49   | 18.12    | 304  | 3.05  | 60.5   | 0.64                    | 1.28        |
| 44.29  | 514  | 80.20        | 3.00   | 218  | 67.74     | 33   | 11.50    | 263  | 2.36  | 76.7   | .76                     | 1.63        |
| 45.14  | 513  | 78.03        | 3.72   | 242  | 58.12     | 24   | 11.66    | 247  | 2.12  | 81.5   | .88                     | 1.75        |

## EXAMPLE 5

A low grade Florida phosphate feed containing about 31% B.P.L. was conditioned with various amounts of talloel soap and talloel and floated as

in Example 4 with only a single cleaning of the concentrate. Various amounts of slime were deliberately added to the feed and it will be noted that the slime produces no adverse effect. The results appear in the following table:

Table VI

| Feed   |      | Concentrates |        |      | Middlings |      | Tailings |      | Ratio | Recov. | Lbs. slime/ton feed added |  |
|--------|------|--------------|--------|------|-----------|------|----------|------|-------|--------|---------------------------|--|
| B.P.L. | Gms. | B.P.L.       | Insol. | Gms. | B.P.L.    | Gms. | B.P.L.   | Gms. |       |        |                           |  |
| 30.99  | 500  | 76.17        | 6.50   | 179  | 42.87     | 23   | 2.93     | 298  | 2.70  | 88.1   | 0.45                      |  |
| 31.11  | 499  | 76.26        | 6.40   | 176  | 43.39     | 27   | 3.15     | 296  | 2.84  | 88.3   | .90                       |  |
| 30.61  | 499  | 75.56        | 6.80   | 180  | 32.72     | 26   | 2.80     | 293  | 2.77  | 89.1   | 1.80                      |  |
| 30.91  | 498  | 75.80        | 6.65   | 179  | 39.03     | 25   | 2.69     | 292  | 2.77  | 88.5   | 2.70                      |  |
| 30.81  | 498  | 76.04        | 6.46   | 177  | 41.19     | 24   | 3.02     | 297  | 2.81  | 87.8   | 4.50                      |  |

described in Example 4 except that the concentrate was cleaned twice. The feed was -48 mesh. The metallurgical results appear in the following table:

An extremely low grade Florida phosphate feed containing about 20% B.P.L. was conditioned and

Table V

| Feed   |      | Concentrates |        |      | Middlings |      | Tailings |      | Ratio | Recov. | Reagents, lbs./ton feed |         |
|--------|------|--------------|--------|------|-----------|------|----------|------|-------|--------|-------------------------|---------|
| B.P.L. | Gms. | B.P.L.       | Insol. | Gms. | B.P.L.    | Gms. | B.P.L.   | Gms. |       |        | Talloel soap            | Talloel |
| 31.02  | 495  | 76.80        | 5.85   | 177  | 32.29     | 41   | 1.57     | 277  | 2.80  | 88.4   | 0.45                    | 1.14    |
| 30.94  | 503  | 75.71        | 6.30   | 188  | 33.32     | 28   | 1.90     | 289  | 2.70  | 90.6   | .33                     | 1.25    |
| 31.35  | 500  | 76.91        | 6.00   | 182  | 36.46     | 27   | 2.38     | 291  | 2.75  | 89.2   | .22                     | 1.38    |
| 31.02  | 499  | 76.36        | 5.60   | 178  | 38.06     | 30   | 2.66     | 291  | 2.80  | 87.9   | .11                     | 1.51    |
| 31.13  | 505  | 73.00        | 5.25   | 202  | 17.85     | 28   | 1.72     | 275  | 2.50  | 93.8   | .22                     | 1.00    |
| 31.28  | 509  | 72.91        | 4.75   | 198  | 32.38     | 25   | 2.38     | 286  | 2.57  | 90.7   | .22                     | .74     |

## EXAMPLE 6

A low grade feed as described in the foregoing example was conditioned with 0.22 pound of talloel soap and talloel oil. The feed was -48 mesh and the concentrate was cleaned twice. The results appear in the following table:

Table VII

| Feed   |      | Concentrates |        |      | Middlings |      | Tailings |      | Ratio | Recov. | Reagents, lb./ton feed |         |             |
|--------|------|--------------|--------|------|-----------|------|----------|------|-------|--------|------------------------|---------|-------------|
| B.P.L. | Gms. | B.P.L.       | Insol. | Gms. | B.P.L.    | Gms. | B.P.L.   | Gms. |       |        | Talloel soap           | Talloel | Coconut oil |
| 20.41  | 504  | 74.14        | 7.75   | 121  | 20.10     | 32   | 1.92     | 351  | 4.17  | 87.1   | 0.22                   | 1.25    |             |
| 19.71  | 500  | 74.44        | 6.90   | 103  | 41.53     | 23   | 2.25     | 364  | 4.85  | 77.9   | .22                    | 1.13    |             |
| 18.30  | 500  | 78.27        | 2.95   | 87   | 57.72     | 29   | 3.04     | 384  | 5.75  | 70.5   | .34                    | -----   | 1.29        |

7  
EXAMPLE 8

A Florida pebble phosphate feed from a different deposit from that used in the foregoing example was conditioned with an ordinary soap, sodium silicate and coconut oil in varying amounts, and single cleaning of the rougher concentrate was employed. The conditioning procedure was the same as in the foregoing examples and the flotation time was also the same. The 10 results appear in the following table:

2. A method of beneficiating phosphate ore by froth flotation which comprises conditioning the phosphate ore with from about 0.1 to about 1.3 lbs. per ton of a talloel soap and an amount of 5 coconut oil at least substantially equal in weight to the soap, and subjecting the conditioned ore to froth flotation, removing a froth concentrate rich in phosphate and a tailing poor in phosphate.

3. A method of beneficiating phosphate ore by 10 froth flotation which comprises conditioning the phosphate ore with from about 0.1 to about 1.3

Table VIII

| Feed   |      | Concentrates |        |      |        | Middlings |        | Tailings |       | Midds. loss |       | Midds. rec. |       | Lbs./ton feed |       |       | Lbs./ton conc. |       |  |
|--------|------|--------------|--------|------|--------|-----------|--------|----------|-------|-------------|-------|-------------|-------|---------------|-------|-------|----------------|-------|--|
| B.P.L. | Gms. | B.P.L.       | Insol. | Gms. | B.P.L. | Gms.      | B.P.L. | Gms.     | Ratio | Rec.        | Ratio | Rec.        | Vege- | Sodi-         | Coco- | Vege- | Sodi-          | Coco- |  |
| 33.73  | 522  | 73.74        | 6.80   | 201  | 26.30  | 37        | 6.38   | 284      | 2.60  | 84.2        | 2.46  | 89.7        | 1.29  | 0.86          | 1.22  | 3.34  | 2.23           | 3.16  |  |
| 33.40  | 520  | 74.86        | 4.85   | 165  | 51.45  | 35        | 10.14  | 320      | 3.15  | 71.0        | 2.78  | 81.3        | .86   | .86           | 1.22  | 2.72  | 2.72           | 3.87  |  |

## EXAMPLE 9

Phosphate feed from the same deposit as Example 8 was conditioned and floated using a fish acid soap, sodium silicate and coconut oil. Conditioning and flotation conditions were the same as in Example 8 and the metallurgical results appear in the following table:

25 lbs. per ton of a talloel soap and an amount of palm oil at least substantially equal in weight to the soap, and subjecting the conditioned ore to froth flotation, removing a froth concentrate rich in phosphate and a tailing poor in phosphate.

4. A method of beneficiating phosphate ore by 30 froth flotation which comprises conditioning the phosphate ore with from about 0.1 to about 1.3

Table IX

| Feed   |      | Concentrates |        |      |        | Middlings |        | Tailings |       | Midds. loss |       | Midds. rec. |      | Lbs./ton feed |       |      | Lbs./ton conc. |       |  |
|--------|------|--------------|--------|------|--------|-----------|--------|----------|-------|-------------|-------|-------------|------|---------------|-------|------|----------------|-------|--|
| B.P.L. | Gms. | B.P.L.       | Insol. | Gms. | B.P.L. | Gms.      | B.P.L. | Gms.     | Ratio | Rec.        | Ratio | Rec.        | Fish | Sodi-         | Coco- | Fish | Sodi-          | Coco- |  |
| 34.04  | 520  | 76.01        | 4.25   | 176  | 54.41  | 34        | 7.98   | 310      | 2.95  | 75.6        | 2.61  | 86.0        | 1.29 | 0.86          | 1.22  | 3.82 | 2.55           | 3.63  |  |

## EXAMPLE 10

A further portion of the phosphate feed of Examples 8 and 9 was conditioned with talloel soap and palm oil, conditioning and flotation procedures being the same as in the two foregoing examples. Metallurgical results are as follows:

45 lbs. per ton of a talloel soap and an amount of taloil at least substantially equal in weight to the soap, and subjecting the conditioned ore to froth flotation, removing a froth concentrate rich in phosphate and a tailing poor in phosphate.

BRUCE DONALDSON CRAWFORD,  
DAVID WALKER JAYNE, JR.

Table X

| Feed   |      | Concentrates |        |      |        | Middlings |        | Tailings |       | Midds. loss |       | Midds. rec. |         | Lbs./ton feed |         |      | Lbs./ton conc. |  |  |
|--------|------|--------------|--------|------|--------|-----------|--------|----------|-------|-------------|-------|-------------|---------|---------------|---------|------|----------------|--|--|
| B.P.L. | Gms. | B.P.L.       | Insol. | Gms. | B.P.L. | Gms.      | B.P.L. | Gms.     | Ratio | Rec.        | Ratio | Rec.        | Talloel | Palm          | Talloel | Palm |                |  |  |
| 34.36  | 516  | 73.94        | 7.70   | 211  | 27.31  | 28        | 4.92   | 277      | 2.45  | 68.0        | 2.34  | 92.3        | 1.22    | 1.80          | 2.97    | 4.40 |                |  |  |

The results obtained in Examples 8 to 10 are not comparable with results of Examples 1 to 7 because the phosphate feed was from a different deposit. In general the feed used in Examples 1 to 7 is somewhat better in its behavior in flotation under the process of the present invention.

We claim:

1. A method of beneficiating phosphate ore by froth flotation which comprises conditioning the phosphate ore with from about 0.1 to about 1.3 lbs. per ton of a talloel soap and an amount of saponifiable oil at least substantially equal in weight to the soap, and subjecting the conditioned ore to froth flotation, removing a froth concentrate rich in phosphate and a tailing poor in phosphate.

## REFERENCES CITED

The following references are of record in the file of this patent:

## UNITED STATES PATENTS

| Number    | Name               | Date           |
|-----------|--------------------|----------------|
| 1,547,732 | Broadbridge et al. | July 28, 1925  |
| 2,165,268 | Vogel-Jorgensen    | July 11, 1939  |
| 1,986,816 | Hasselstrom        | Jan. 8, 1935   |
| 2,014,406 | Weed               | Sept. 17, 1935 |
| 2,156,245 | Mead et al.        | Apr. 25, 1939  |